

## UNITED STATES PATENT OFFICE

2,014,294

PROCESS FOR THE PRODUCTION OF  
ACETONEKoloman Róka and Karl Wiesler,  
Constance, GermanyNo Drawing. Application May 11, 1933, Serial No.  
670,619. In Germany November 14, 1926

17 Claims. (Cl. 260—134)

This invention relates to the production of acetone from acetylene, and is, in part, a continuation of our earlier application Serial No. 228,685, filed October 25, 1927.

5 Although the preparation of acetone by reacting acetylene ( $C_2H_2$ ), and water vapor at high temperatures has been effected, the process has never been satisfactory from a commercial standpoint. The yields of the desired ketone have always been too low to permit that economy which is requisite to a process of satisfactory commercial practicability. Moreover, the catalysts employed in the known processes have always lost their efficacy after a relatively small period of continuous use, thus necessitating the frequent renewal of these contact masses. This has added to the expense of producing the acetone and has deferred manufacturers from utilizing the process commercially. Moreover, the inconvenience of frequently replacing the catalyst in the reaction vessels and the irregularity caused by such replacement have prevented the process from becoming a reliable commercial method for the manufacture of acetone.

20 Our invention has for one of its objects a process for the production of acetone from acetylene and steam which will result in yields of the desired ketone in such amounts that the process can be carried out efficiently in the commercial manufacture of this chemical compound. Moreover, our process is one which permits continuous production in the large quantities necessary for efficient factory operation, since the catalytic materials we employ suffer no appreciable decrease in catalytic power regardless of the duration of the reaction period. Another object of our invention is the avoidance of frequent replacement of the contact mass by the use of catalytic mixtures which maintain their activity for practically unlimited periods.

25 Still another purpose of our novel process is the production of acetone by a procedure which will not be affected by catalytic poisons present in the acetylene and will not require an extremely large excess of water vapor or steam. These features are important because they make possible in our process the use of ordinary acetylene without the necessity of purifying this gas to a high degree. By reducing the quantity of steam required, the process is carried out with a maximum economy. If it were necessary to free the acetylene from impurities, the cost would be increased to such a degree that the process would be commercially impractical. It is clear, therefore, that in the process disclosed herein, this enormous

expense accompanying prior procedures has been eliminated.

Another object of our process is the reaction of the acetylene and steam at a lower temperature than was formerly usual in this type of reaction. While the temperatures that we employ have occasionally been utilized in the past, it is desired to point out that it was customary in general to employ a higher temperature of reaction. The lower temperature required in our process results in further important economy of operation.

Our process depends on a principle which we are the first to employ in a reaction of this type. This principle, which involves the adjustment of the catalyst so as to yield a partial oxygen pressure within certain fixed limits, has never before been applied in the commercial production of acetone. This method of adjustment will be fully described later on in this specification.

Reference may be made at this time to Austrian Patent No. 88,631 which describes the method which was known prior to the invention of the applicants but which never went into commercial use. The process of this patent requires that the acetylene be freed of catalytic poisons and will result in acetone in appreciable amounts only when water vapor is present in forty times the quantity theoretically required for the reaction. Under some conditions a yield of 40% of acetone has been obtained, but this yield is too low to permit the method to be used commercially to any great extent.

The process of the Austrian patent suggests the use of catalysts which are as rich as possible in iron oxide. These are to be obtained by precipitating iron oxide and pressing the precipitated material into lumps. When only small quantities of  $Fe_2O_3$  are present, as in a catalyst prepared by applying iron oxide to a contact carrier material, the formation of acetone is considerably reduced, the main product consisting of acetaldehyde. For this reason the Austrian patent states that natural iron ores and their by-products such as clay iron-stone ( $FeCO_3$ ), clay, and shale, sparry iron ore, and waste from pyrites may be used as catalysts with the production of acetone in yields from 25 to 50%. It is to be noted that the yield is relatively low and that purified acetylene and a large excess of water vapor are essential to success.

The applicants have made thorough studies of the entire problem with a view to improving the process so that yields of acetone approaching the theoretical may be obtained. As a result of these investigations, the discovery was made that the activity of the main catalysts employed in the

process of the Austrian specification, the iron oxide compounds therein mentioned, could be increased and prolonged to a very considerable extent by the addition of one or more cooperating auxiliary catalysts. Among these auxiliary catalysts may be mentioned metallic iron, manganese oxide, aluminum oxide, barium carbonate, zinc carbonate, lime, and magnesia. It may be pointed out that the carbonates of barium, calcium, and zinc are easily reduced during the process and yield the oxides of the metals which together with the iron oxide constitute the catalytic masses. For this reason the applicants have made further investigations with a view to determining the essential nature of the catalytic materials necessary. These studies led to the following astounding results.

We found after considerable experimentation that a mixture of metallic compounds provided a catalytic agent of unusual stability and activity. These mixtures of metallic compounds, preferably metal-oxygen compounds, gave very satisfactory results over unusually long periods of time and especially satisfactory results were obtained when the partial oxygen tension of the mixture was adjusted within certain values as more fully described subsequently in this disclosure. While all metallic compounds containing oxygen are suitable, we have found that metal oxides, or salts which yield the oxide of the respective metals under the conditions of the process, such as carbonates, acetates, tartrates, or other similar salts will yield the most satisfactory results.

The prepared catalytic mixture may comprise a heavy metal carrier and a metal-oxygen compound. For this latter compound either an oxide of a heavy metal or an oxide of a light metal or both may be used. Specifically, a heavy metal oxide and a light metal oxide may be employed in conjunction with some type of metal carrier. Of course, in place of the oxides, any metal oxygen compound may be used with more or less success, and metal oxygen compounds which yield the oxide under the conditions of the process will be found to give excellent results.

Two metal oxides may be admixed to form the catalytic material and the partial oxygen tension of the mixture may or may not be adjusted as hereinafter described. A mixture of a heavy metal oxide and a light metal oxide, or a heavy metal oxide and a light metal carbonate has been found to constitute a stable and efficient catalyst. A mixture including a heavy metal oxide and another heavy metal oxide, or a heavy metal oxide and a heavy metal carbonate is an excellent contact mass. Mixtures of heavy metal oxides and a metal; or light metal oxides and a metal; or a mixture of a light metal oxide and a heavy metal oxide with a metal carrier have all been tried with success. Other metal oxygen compounds may be used instead of the oxides in these specific mixtures and the employment of a salt which will yield a metal oxide under the conditions of the process is the full equivalent of the use of the oxide. Mixtures of three, four or more metallic oxygen compounds have been tried with very satisfactory results and some examples of processes which employ such catalytic mixtures are more fully described below.

We have made many experiments on a commercial and semi-commercial scale with iron-oxygen compounds, such as iron oxide or any compound yielding iron oxide under the conditions of the process in conjunction with a metal, such

as iron, and an auxiliary oxygen-containing catalyst such as manganese oxide, barium carbonate, barium oxide, and similar oxidic materials. The results have always been very satisfactory. Advantageous results are often attained by the employment of the principal and main catalysts in conjunction with a metallic carrier such as iron or superficially oxidized iron. Rusty iron shavings, for example, may be coated with a thin layer of manganese oxide, zinc oxide, or any other 10 metallic oxide.

As examples of heavy metals which may be used in the process as carriers for other catalytic materials, iron, manganese, nickel, cobalt, platinum, molybdenum and tungsten have been found 15 suitable. Of course, other metals can be used as support for the metal oxygen compounds with equal success and we do not desire to be limited to any class or group of metals.

When we have referred to heavy metal oxides 20 in the foregoing description we have had in mind the following specific oxidic materials which will be found suitable. The list is merely illustrative of this type of metal-oxygen compound and is by no means to be interpreted as limiting the 25 catalytic materials which may be employed in our process. The roman numeral after each of the metals indicates the group of the periodic table in which the metal is found. These heavy metal oxides are those of the following metals, iron 30 VIII, cobalt VIII, nickel VIII, manganese VII, molybdenum VI, tungsten VI, bismuth V, antimony V, lead IV, tin IV, cadmium II, mercury II, copper I, and silver I.

As light metal oxides, compounds yielding the 35 oxides of any of the following light metals are suggested and will be found suitable. Here again the list is merely illustrative and not restrictive. The roman numeral again indicates the group of the periodic table in which the metal is clas- 40 sified. These oxides of light metals are sodium II, potassium I, magnesium II, calcium II, zinc II, barium II, and aluminum III.

It is to be understood, of course, that compounds which readily yield the metallic oxide 45 under the conditions of the process may be used in place of the oxide itself, for indeed this amounts to a use of the metallic oxide. Carbonates, nitrates, and acetates are very readily reduced to the oxides and may efficiently be em- 50 ployed in the process. Carbonates such as those of zinc, magnesium, barium, and calcium are usually more readily obtained than the oxides and may be readily used as the equivalent of the metal oxides. The appended examples furnish 55 some illustrations of the use of nitrates, acetates and carbonates for the purpose of furnishing a metal oxide to the process.

Particular mixtures of certain metallic com- 60 pounds have been found to yield catalysts of high efficiency and unusually long life. Thus a mixture of an oxide of manganese such as manganese dioxide and an iron oxide (either  $Fe_2O_3$  or  $Fe_3O_4$ ) has been found particularly successful in our process. A mixture of iron oxide and a car- 65 bonate of a heavy metal such as magnesium, lead, or bismuth may be utilized. Mixture of three or more oxidic materials such as the oxides of zinc, iron, and manganese, or those of magnesium, iron, zinc, and manganese, or other combina- 70 tions have been found very suitable in the process. Oxidic mixtures and metallic iron, or a single metal oxide and metallic iron (such as an iron reaction pipe) have been found to furnish contact masses of unusual stability and efficiency. 75

A fundamental principle which may be employed in the selection of oxidic mixtures is to add mix the substances so that a partial pressure of oxygen within the limits of  $10^{-25}$  atmospheres and  $10^{-30}$  atmospheres will result. While not limited in range to the range defined by these two partial dissociation values, it will be found that our process yields excellent results within these ranges when the process is carried out at

10  $400^{\circ}$  C. or  $500^{\circ}$  C. with five to ten parts of water vapor to one part of acetylene.

As explained above, it may be advisable under some circumstances to select and arrange the catalysts so that under the conditions of the process an oxygen tension is produced which falls within the limits given above. This may be accomplished in any manner well known to the skilled chemist. For convenience, an explanation of the method and a reference to the literature 15 is now given in some detail. Partial dissociation values and adjustment of the components of mixtures to attain any given predetermined oxygen tension may be readily carried out in accordance with the following procedure.

20 The process can perhaps best be explained by the use of a specific example. In one aspect of our process one mole of acetylene and ten moles of steam are caused to react at a temperature of  $500^{\circ}$  C. in the presence of a catalytic mixture 25 which may be composed of iron oxide with the addition of other suitable metal oxygen compounds. The determination of the oxygen tension naturally resolves itself into two problems, first, the determination of the oxygen tension in 30 the gaseous phase due to the presence of water vapor in the reaction, and second, the determination of the oxygen tension of the solid phase. The oxygen tension in the solid phase is due to the presence of the solid metal oxygen compounds 35 as catalytic materials, and it is the adjustment 40 of this oxygen tension which forms the practical problem to be solved in these theoretical considerations.

#### A. Oxygen tensions in the gaseous phase

45 The reaction occurring in the process of this application is expressed by the following formula:



50 However, in order to obtain satisfactory yields, we have found that two moles of acetylene should preferably be reacted with an excess of 55 water vapor so that for every two moles of acetylene there is present a quantity of steam amounting to twenty moles. When this condition is inserted in the chemical equation, the following equation results:



55 From this equation it is therefore apparent that if  $p$  expresses an oxygen tension or partial pressure, the following ratio represents the conditions in the reaction vessel:

$$(3) \quad \frac{p_{\text{H}_2\text{O}}}{p_{\text{H}_2}} = \frac{17}{2} = 8.5$$

70 From considerations of physical chemistry, the value of the constant  $K'$  is expressed as follows:

$$(4) \quad K' p_{\text{H}_2\text{O}} = \frac{p_{\text{H}_2\text{O}}^2 \cdot p_{\text{O}_2}}{p_{\text{H}_2\text{O}}^2}$$

75 The numerical value of this constant can be

determined very accurately by the equation given by Siegel, see Zeitschrift für Physikalische Chemie, volume 87, page 641 (1914).

(5)

$$\log K = \frac{-24900}{T} + 1.335 \log T - 9.65 \times 10^{-5} T + 1.37 \times 10^{-7} T^2 - 6.65 \times 10^{-11} T^3 + 1.907 \times 10^{-18} T^4 - 1.08$$

For a temperature of  $500^{\circ}$  C.,  $T$  is  $773^{\circ}$  since  $T$  represents the absolute temperature for these conditions.  $K' p_{\text{H}_2\text{O}}$  has a numerical value of  $3.33 \times 10^{-30}$ .

Substituting this value in Equation (4) there results:

$$(6) \quad p_{\text{O}_2} = K' p_{\text{H}_2\text{O}} \times \frac{p_{\text{H}_2\text{O}}^2}{p_{\text{H}_2}^2} \\ = 3.33 \times 10^{-30} \times (8.5)^2 \\ = 0.25 \times 10^{-27}$$

#### B. Oxygen tensions of the solid phase

The oxygen tension of the solid phase catalysts may be computed from the heat of formation which is given by the Nernst equation. See Treadwell's article, Zeitschrift Electro Chemie, 25 volume 22, page 414 (1916). See also Pollitzer "Berechnung der Chem. Affinitäten nach dem Nernst'schen Wärme-Theorem. The equation is as follows:

$$(7) \quad \log p = \frac{-Q}{4.571T} + 1.75 \log T + 2.8$$

In this equation  $Q$  represents the heat of formation.

1. In order to ascertain the oxygen tensions of  $\text{Fe}_2\text{O}_3$  at different temperatures, a knowledge of the heat of formation arising from the reaction:



is necessary. Treadwell has determined that at 40 room temperature  $Q=90,400$  calories.

At  $1000^{\circ}$  C. Treadwell deduces as a result of his potential measurements that  $Q=91,000$  calories. If we use the mean value of Treadwell's measurements for the value of  $Q$  in the Nernst equation, 45 we find:

$$(9) \quad p_{\text{O}_2} = 1.5 \times 10^{-18}$$

2. For  $\text{Fe}_3\text{O}_4$  the oxygen tension at  $500^{\circ}$  C. can be similarly determined. The values result as follows:

$$1.2 \times 10^{-34} \\ 4.4 \times 10^{-34} \\ 1.4 \times 10^{-34}$$

It will be seen that these measurements do not 55 agree very closely. The variance is the result of use of different values for the heat of formation. The three values for the heat of formation which result in the three different values for

$p_{\text{O}_2}$

of  $\text{Fe}_3\text{O}_4$  are those of:

a. Wöhler & Günther Zeitschrift El. Ch. 29, 276

(1923)

b. Mixter Sill. Journal (4) 40, 23 (1915)

c. Treadwell Zeitschrift El. Chem., vol. 22, 414

(1916).

It is evident that the iron oxide  $\text{Fe}_3\text{O}_4$  possesses a much lower oxygen tension than  $\text{Fe}_2\text{O}_3$  since it can be considered to be formed by the addition of  $\text{FeO}$  to  $\text{Fe}_2\text{O}_3$ . In fact, the oxygen tension decreases as the  $\text{FeO}$  content rises. For experimental results the Examiner should refer to Sosman and Hostetler, Journal of the American Chemical Society, 38, pages 807 and 1188 (1916). Numeri- 70 75

cal values will be found in the Physical Chemical Tabellen by Landolt-Bärnstein, vol. 2, page 1405.

If it should be desired to adjust the oxygen tension to a value of  $0.25 \times 10^{-7}$  atmospheres, as in the process described in this application, it is at once apparent that this value is attained by the use of a mixture of  $Fe_2O_3$  and  $FeO$ , with a lower  $FeO$  content than that which corresponds to the  $FeO$  content in the oxide  $Fe_3O_4$ . The percentage of  $FeO$  in the mixture is then ascertained by experimental determination of the oxygen tension of several different mixtures. This experimental determination of the oxygen tension may be done by several methods, one of which, for example, is the method disclosed in the Treadwell article referred to above. This involves determination of the oxidation potential  $E$  and by use of the following equation

$$20 \quad p_{O_2}$$

can be computed:

$$(10) \quad E = -5T \times 10^{-8} \times \log p_{O_2}$$

25 3. In order to determine the oxygen tension of the mixture comprising the water vapor and the oxides, a process analogous to the process of Wöhler and Günther may be followed. This method is given in the Zeitschrift für El. Ch., volume 29, page 276 (1923). This value may be combined with the value arising from dissociation of water vapor, and the oxygen tension

$$35 \quad p_{O_2} = K' \frac{X}{p_{H_2O}}$$

represents the constant resulting from homogeneous water vapor dissociation, and  $K$  represents the constant of the heterogeneous system. 40 By using the Siegel equation the values obtained for the constant

$$K' \frac{X}{p_{H_2O}}$$

45 are very accurate values. However, by the use of the Nernst equation of approximation, values of sufficient accuracy are obtained.

4. The heterogeneous  $CO_2$  values are combined in a similar way with the homogeneous carbon dioxide values, and this permits a computation 50 of the oxygen tensions. See K. Hofmann, Zeitschrift für El. Ch., 31, 172, (1925).

A few determinations of this kind are sufficient to ascertain the composition of the mixture which 55 will possess the desired oxygen tension. It is believed that it is quite clear how the concentration of  $FeO$  should be changed in the mixture and that the oxygen tension for each mixture containing a certain percentage of  $FeO$  can be very readily ascertained.

60 It is also apparent that this method can be applied not only when using the iron oxide  $FeO$  in the mixture, but also when other metallic oxides are admixed. If it is required to diminish the oxygen tension of, for example,  $Fe_2O_3$ , iron oxide, a metal oxide such as zinc oxide, aluminum oxide, calcium oxide, any of the manganese oxides, or other metal oxygen compounds can be very readily substituted for the ferrous oxide.

65 The particular oxygen tension to be maintained is readily derivable from and is correlated with the degree of dissociation of water vapor as determined by the temperature and dilution of the acetylene under the conditions at which our process is carried out. It will be found that adjustment of the partial oxygen tensions within the

range specified results in catalysts of particularly long life.

Our process is advantageously carried out with more than four parts by volume of water vapor or steam to one part by volume of acetylene. 5 When five to ten parts by volume of water vapor to one part of acetylene are employed with catalysts which have been adjusted to a predetermined oxygen tension the results are excellent. An excess above fifteen parts of water vapor or 10 steam to one part of acetylene should, in general, be avoided, as such an excess is unnecessary and uneconomical.

The temperature at which our process is carried out with highest efficiency is somewhere between 250° C. and 750° C. In general main operating temperatures between 350° C. and 600° C., and preferably within the range of 450° C. to 550° C. will be found to give most satisfactory results. It has been frequently found advantageous to start the process at a comparatively low temperature and then increase the temperature either gradually or in stages to a higher value. In this way it is possible to maintain the oxygen tension continually within the limits satisfactory for the reaction.

20 Specific examples of our process are appended hereto, and further details of the conditions of operation will be found therein. It is to be understood, of course, that these operating conditions are merely illustrative and our invention is by no means limited to the precise process as defined in these examples.

25 It may be mentioned here that ores have in general been found unsuitable for catalytic masses, although they may frequently form an initial material from which a satisfactory catalyst may be produced. The ore disclosed as suitable in the Austrian patent referred to has been found to yield unsatisfactory and uncertain results. When the process is carried out as described in this patent, the catalyst was found to have lost its efficiency after use amounting to three days. The catalytic masses disclosed in this specification as our invention have been 45 found to be of undiminished activity after thirty days or more of continuous use.

30 As examples of our novel process, I submit the following:

#### Example I

35 Superficially oxidized iron shavings were heated in an iron pipe to about 500° C. to form the catalyst. Over the catalytic agent thus resulting, a mixture of acetylene and water vapor in the molecular proportion of 1:10 was passed. The vapors issuing from the heated reaction pipe were cooled and resulted in a dilute solution of acetone, the yield of this ketone amounting to 83% of the theoretical quantity as calculated from the acetylene employed in the process.

40 The non-condensable fraction contained 7.6% by volume of unchanged acetylene. The yield of the desired ketone, acetone, was indeed very satisfactory, since quantitatively it amounted to 65 94% of the theoretical, based on the quantity of acetylene entering into the reaction.

#### Example II

45 Iron shavings were coated with iron oxide and manganese dioxide and introduced into a reaction pipe. Over this catalytic material a mixture of one part of acetylene and ten parts of water vapor, by volume, were passed at 475° C. The vapors issuing from the reaction pipe were con- 75

densed. The acetone present in the condensate amounted to 95% of the theoretical quantity calculated on the basis of the acetylene employed in the process. At the end of thirty days the 5 activity of the catalyst had not been impaired nor had its vigor been appreciably diminished.

*Example III*

10 Iron shavings were provided with a superficial coating of iron oxide and barium carbonate, and introduced into an iron reaction pipe. A mixture of acetylene and water vapor in the ratio of one part  $C_2H_2$  to ten parts of water, by volume, was passed through the reaction pipe at a temperature of  $470^\circ C$ . Upon condensation of the issuing vapors, acetone in the amount of 90% of the maximum yield possible, calculated on the 15 quantity of acetylene used, was obtained.

*Example IV*

20 Naturally occurring manganese dioxide was impregnated with zinc acetate in the amount of 25% of its weight. The manganese dioxide, thus impregnated was subjected to a current of nitrogen at  $600^\circ C$ . for the purpose of decomposing the material. Over the oxidic mixture thus produced, a mixture of acetylene and steam was led. The process, which was carried out at  $420^\circ C$ ., was regulated so that a mixture of 9.9 liters of acetylene and 119 grams of steam, per liter of catalyst, 25 was conducted over the catalytic oxidic material every hour.

25 After four hours a yield of 75.3% of acetone was obtained. The quantity of acetylene which did not enter into the reaction and was regained unchanged amounted to 9.7%, while 8.8% of the acetylene supplied was converted to carbon dioxide, as a result of complete combustion.

*Example V*

30 Granular pumice stone was impregnated with zinc acetate, iron nitrate, and manganese acetate. The materials were employed in the following proportions, 800 grams of pumice stone requires 35 135 grams of zinc acetate, 148 grams of iron nitrate and 15 grams of manganese acetate. The pumice stone, thus impregnated, constituted the catalyst.

35 Over this catalytic agent a mixture of acetylene and steam was conducted at a temperature of  $485^\circ C$ . Acetylene and steam were admixed and led over the impregnated pumice stone at the rate of 10.3 liters of acetylene and 123 grams of steam per liter of catalyst per hour.

40 A yield of 68.2% acetone was obtained at the conclusion of the experiment, at the end of four hours. Acetylene in the amount of 20.6% passed through unchanged, while 4.6% of acetone was converted to carbon dioxide.

*Example VI*

45 The catalyst was prepared by impregnating 920 grams of granular magnesite ( $MgCO_3$ ) with a concentrated solution containing 125 grams of iron nitrate. The magnesite was then heated and during the process it was impregnated with a second solution containing 68 grams of zinc acetate, 125 grams of iron nitrate, 7.5 grams of manganese acetate and 10 grams of magnesium acetate. This resulted in the precipitation of the respective metallic hydroxides, whereupon the catalytic material was filtered off and dried.

50 Over this contact mass, acetylene and steam were passed, at the rate of 11.3 liters of acetylene, 55 and 136 grams of steam per liter of catalyst, per

hour. The process was continued for four hours. A yield of acetone of 77.4%, calculated on the basis of the quantity of acetylene supplied, was obtained. The acetylene recovered in unchanged form from the issuing vapors was 8.3% of the 5 total, which 5.9% of the acetylene supplied to the process was lost by conversion to carbon dioxide.

*Example VII*

10 The catalyst was prepared by impregnating oxidized iron sponge with a solution containing 90 grams of zinc acetate for every kilogram of iron sponge. The process was carried out by conducting a mixture of acetylene and steam at the rate of 10.8 liters of acetylene and 138 grams of 15 steam per liter of catalyst, per hour, over the contact mass at a temperature of  $425^\circ C$ . The process was continued for 218 hours. A yield of 83.7% of acetone was obtained, calculated on the basis of the acetylene supplied to the reaction. 20 The issuing gases showed 4.2% of carbon dioxide and 9.1% of unreacted acetylene.

*Example VIII*

25 The catalyst was prepared by impregnating oxidized iron sponge as described in Example VII. The acetylene and steam were supplied at the rate of 8.9 liters of acetylene and 122 grams of steam per liter of contact, per hour. At the end of four hours a yield of 88.5% of acetone, based on the 30 acetylene supplied to the reaction, was obtained. The unconverted acetylene amounted to 6.9% and the issuing gases contained 1.7% of carbon dioxide.

*Example IX*

35

40 Oxidized iron sponge was impregnated with zinc acetate, iron nitrate, and manganese acetate until the metals impregnated, calculated as the respective metal oxides, amounted to 4.2% of the catalyst. The metals zinc, iron and manganese were present in the ratio, 4:1.5:1. Over this catalyst a mixture of acetylene and steam was conducted at a temperature of  $440^\circ C$ . The mixture consisted of 9.5 liters of acetylene and 114 45 grams of steam per liter of catalyst per hour. At the end of 284 hours, a yield of acetone of 89.7% of the theoretical, based on the quantity of acetylene supplied, had been obtained. The quantity of acetylene passing through unchanged 50 was 6.3% and 1.6% of carbon dioxide was present in the issuing vapors.

*Example X*

55 Over a catalytic mass prepared as in Example IX, a mixture of acetylene and steam was passed at  $440^\circ C$ . The mixture contained 9.5 liters of acetylene and 114 grams of steam per liter of catalyst per hour. At the end of four hours the yield of acetone was 84.8%, based on the quantity 60 of acetylene used in the reaction. The unchanged acetylene was 4.6% of the total, and the issuing gases contained carbon dioxide corresponding to 0.24% of the acetylene. This represented a loss of acetylene due to too complete a combustion. 65

*Example XI*

70 Over a catalyst prepared as in Example IX, a mixture of acetylene and steam was conducted at a temperature of  $450^\circ C$ . 19.1 liters of acetylene 70 and 230 grams of steam were led over the catalyst every hour for every liter of the contact mass. After 76 hours, a yield of 85% acetone was obtained, calculated on the quantity of acetylene employed. 10% of the acetylene passed through 75

unchanged, while the waste products included 3.6% of carbon dioxide.

*Example XII*

5 Oxidized iron sponge material was impregnated with zinc acetate, iron nitrate and magnesium acetate until the resulting metallic oxides amounted to 4.3% of the weight of the catalyst. The three metals added by impregnation were 10 present in the ratio 12:1.3:1. Over this catalyst a mixture of acetylene and steam was conducted at 440° C. The reacting mixture was passed over the contact mass at a rate of 9.8 liters of acetylene and 118 grams of steam per liter of catalyst per 15 hour. At the end of 124 hours a yield of 91% of acetone had been obtained, calculated on the basis of the quantity of acetylene supplied. The unchanged acetylene in the exhaust gases amounted to 6.3%, and 2.1% of the acetylene supplied was lost through complete combustion to carbon dioxide.

*Example XIII*

25 Over a catalyst prepared as in Example XII, a mixture of acetylene and steam was passed at a temperature of 440° C. The acetylene and steam mixture was fed at a rate of 9.8 liters of acetylene and 118 grams of steam per liter of catalyst per 30 hour. At the end of four hours, the acetone yield was 93.7% of the quantity of acetylene supplied. The unconverted acetylene was 5.3% of the total, and 1.2% of  $C_2H_2$  was lost as carbon dioxide.

Having thus described the invention, what we 35 claim as new and desire to secure by Letters Patent of the United States is:

1. A process for the production of acetone which comprises passing a gaseous mixture of acetylene and steam over a catalyst comprising essentially at least one substance selected from the group consisting of metal oxides and metal 40 oxygen compounds which readily yield the oxide under the reaction conditions, the said catalyst having the partial pressure of oxygen within the range of  $10^{-25}$  to  $10^{-32}$  atmospheres.

2. A process for the production of acetone which comprises passing a gaseous mixture of acetylene and steam in approximately the proportions, by volume, of one part of acetylene to 5 to 15 parts of steam over a catalyst comprising 45 essentially at least one substance selected from the group consisting of metal oxides and metal oxygen compounds which readily yield the oxide under the reaction conditions, the said catalyst having the partial pressure of oxygen within the range of  $10^{-25}$  to  $10^{-32}$  atmospheres.

3. A process for the production of acetone which comprises passing a gaseous mixture of acetylene and steam in approximately the proportions, by volume, of one part of acetylene to 50 5 to 15 parts of steam over a catalyst comprising essentially a metal oxide, the temperature of the reaction being maintained between 250° C. and 750° C., the said catalyst having the partial pressure of oxygen within the range of  $10^{-25}$  to  $10^{-32}$  atmospheres.

4. A process for the production of acetone which comprises passing a gaseous mixture of acetylene and steam over a catalyst comprising essentially a plurality of metal oxides, the said 60 catalyst having the partial pressure of oxygen within the range of  $10^{-25}$  to  $10^{-32}$  atmospheres.

5. A process for the production of acetone which comprises passing a gaseous mixture of acetylene and steam over a catalyst comprised 65 essentially of a heavy metal and an oxide of a

light metal, the said catalyst having the partial pressure of oxygen within the range of  $10^{-25}$  to  $10^{-32}$  atmospheres.

6. A process for the production of acetone which comprises passing a gaseous mixture of acetylene and steam over a catalyst comprising essentially a plurality of oxides of heavy metals, the said catalyst having the partial pressure of oxygen within the range of  $10^{-25}$  to  $10^{-32}$  atmospheres.

7. A process for the production of acetone which comprises passing a gaseous mixture of acetylene and steam over a catalyst comprised essentially of iron oxide and a heavy metal carbonate, the said catalyst having the partial pressure of oxygen within the range of  $10^{-25}$  to  $10^{-32}$  atmospheres.

8. A process for the production of acetone which comprises passing a gaseous mixture of acetylene and steam over a mixture having catalytic action and comprising essentially an iron oxide, a heavy metal carbonate and a metal, the said catalytic mixture having the partial pressure of oxygen within the range of  $10^{-25}$  to  $10^{-32}$  atmospheres.

9. A process for the production of acetone which comprises passing a gaseous mixture of acetylene and steam over a mixture having catalytic action and comprising essentially an iron oxide, a light metal carbonate and a metal, the said catalytic mixture having the partial pressure of oxygen within the range of  $10^{-25}$  to  $10^{-32}$  atmospheres.

10. A process for making acetone which comprises passing acetylene and steam, at temperatures within the range of 250° C. to 750° C., over a mixture of a heavy metal oxide and a light metal carbonate, the said mixture having the partial pressure of oxygen within the range of  $10^{-25}$  to  $10^{-32}$  atmospheres.

11. A process for the production of acetone by reacting acetylene and steam, in the presence of a catalytic mixture, comprising the steps of, preparing the catalytic mixture from two metal oxides; and bringing a mixture of one part of acetylene with five to fifteen parts of steam into contact with said catalytic mixture, at temperatures within the range of 300° C. to 600° C.; the said catalytic mixture having the partial pressure of oxygen within the range of  $10^{-25}$  to  $10^{-32}$  atmospheres.

12. A process for making acetone which comprises passing a gaseous mixture of 5 to 15 parts of steam with 1 part of acetylene, in the presence of iron and at temperatures of from 250° C. to 750° C., over a metal oxide, the said metal oxide having the partial pressure of oxygen within the range of  $10^{-25}$  to  $10^{-32}$  atmospheres.

13. A process for making acetone which consists in reacting acetylene and steam at temperatures between 250° C. and 750° C., in the presence of mixtures of substances which contain one heavy metal oxide, one light metal oxide and one metal, the said mixtures having the partial pressure of oxygen within the range of  $10^{-25}$  to  $10^{-32}$  atmospheres.

14. A process for producing acetone consisting in passing acetylene and steam, at temperatures between 250° C. and 750° C., into contact with mixtures of substances which contain one heavy metal oxide catalyst and a substance selected from the group consisting of metal oxides and metal oxygen compounds which readily yield the oxide under the reaction conditions, and which are so compounded that their oxygen tension at 70 75

the temperatures used in the process is near the oxygen partial tension in the reaction mixture containing the oxygen.

15. In the process defined in claim 14, starting 5 the reaction at a temperature near the lower end of the given temperature range and, as the process proceeds, gradually increasing the temperature in order to maintain said oxygen tensions in their proper ratio.

10 16. A process for the production of acetone by reacting acetylene and steam in the presence of a catalytic mixture, consisting in the steps of preparing said mixture from iron oxide and an auxiliary catalyst composed of a substance 15 selected from the group consisting of light metal oxides and light metal oxygen compounds which readily yield the oxide under the reaction conditions in selected proportions, and bringing a mixture of one part of acetylene with five to 20 fifteen parts of steam into contact with said

catalytic mixture at temperatures within the approximate range of 300° C.-600° C., the said selected proportions of the catalytic mixture being such as to maintain the partial pressure of the oxygen in the catalytic mixture within the approximate range of  $10^{-25}$  to  $10^{-32}$  atmospheres. 5

17. A process for the production of acetone which comprises passing a gaseous mixture of acetylene and steam over a mixture having catalytic action and comprising essentially an oxidic 10 mixture selected from the group consisting of the following mixtures: two metal oxides; two metal oxides and a metal; a metal oxide and a metal carbonate; a metal oxide, a metal carbonate and a metal; and a metal oxide and a metal, said 15 catalytic mixture having the partial pressure of oxygen within the range of  $10^{-25}$  to  $10^{-32}$  atmospheres.

KOLOMAN RÓKA.

KARL WIESLER. 20